

1

3,123,472

## ONE-COMPONENT DIAZOTYPE PROCESS AND MATERIAL COMPRISING A DIAZONIUM COMPOUND AND AN ORTHOPHOSPHATE

Johannes Henricus Andreas Wilders and Peter Johannes Nicolaas van den Kroonenberg, Venlo, Netherlands, assignors to Chemische Fabriek L. van der Grinten N.V., Venlo, Netherlands, a corporation of the Netherlands

No Drawing. Filed Nov. 10, 1959, Ser. No. 851,948  
Claims priority, application Netherlands Nov. 10, 1958  
6 Claims. (Cl. 96—49)

The invention relates to one-component diazotype material and more particularly to such material in which the light-sensitive layer has an acid reaction and contains a p-amino benzene diazo compound which has a greater coupling activity than p-diazo ethyl benzylaniline, which is derived from a tertiary amine with only one aryl radical attached directly to the tertiary nitrogen atom, and which carries in the 4-position the diazo group, in the 2-position an alkoxy, aralkoxy or aryloxy group, and in the 5-position a hydrogen atom, a halogen atom, a methyl group or an alkoxy group.

Several of these diazo compounds are known. They are very sensitive to the light of the mercury vapour lamps commonly used in the modern diazotype process. Compounds in which the substituent in the 2-position is an alkoxy group are known, for example, from the Belgian Patent No. 564,343. Diazotype material sensitized with such a diazo compound is extremely suitable for the visual observation of the endpoint of the exposure when copies are made in the light of actinically fluorescent mercury vapour lamps.

Many diazo compounds of the type described above couple more actively than p-diazo ethyl benzylaniline. Their coupling activity, in comparison with that of p-diazo ethyl benzylaniline, can be determined in vitro by measuring the time in which a given proportion (10%, for instance) of the diazo compound to be examined will have coupled in a given molar concentration (0.1 millimolar, for instance) with the coupling component 1-phenyl 3-methyl-5-pyrazolone in a given molar concentration (1.0 millimolar, for instance) in a buffer mixture of a given composition and a given pH at a given temperature.

The compounds coupling more actively than p-diazo ethyl benzylaniline are very suitable for the manufacture of one-component diazotype material which can be developed according to the so-called semi-wet process.

In the diazotype process with semi-wet development, imagewise exposed one-component diazotype material is developed by spreading a thin layer (a layer of 8 g. square meter for instance) of developing liquid, containing one or more azo components and one or more buffer salts, evenly over the surface of the diazotype material. This can be done mechanically, e.g. with the aid of developing apparatus as described in the Dutch Patents Nos. 53,196 and 55,162.

The development always has to be complete, i.e. all of the diazo compound left on the diazotype material after the imagewise exposure has to be converted completely into azo dyestuff, despite the different temperatures occurring in practice, which vary, for example, from 10 to 30° C., and the different humidities of the air occurring in practice, which affect the drying speed of the layer of developing liquid applied on the diazotype material.

Preferably the azo dyestuffs formed should have the same colour even under the said varying conditions.

In semi-wet development under the said varying conditions good results can be achieved with the above-mentioned one-component diazotype material by adapta-

2

tion of the composition and the pH of the developing liquid to the composition of the light-sensitive layer, and to the reactivity of the diazo compound used and of the azo component used.

Good results can thus be obtained with alkaline phloroglucinol developers of a pH between 8.5 and 10.5 which have been buffered sufficiently. They yield brown-coloured azo-dyestuffs in the semi-wet development of one-component diazotype materials which have been manufactured with diazo compounds according to the above definition and the light-sensitive layer of which has the composition that is usual for one-component diazotype materials, containing inter alia a small quantity of acid, such as citric acid, tartaric acid or alum. The desired pH value and the desired buffer capacity of the phloroglucinol developers in question are achieved with the aid of buffer salts such as carbonates, borates, citrates, phosphates, tartrates, and the like. The borate developers described in the United States Patents Nos. 2,657,137 and 2,657,141 are especially suitable.

Phloroglucinol developers showing a stronger or weaker alkaline reaction than those with pH between 8.5 and 10.5 are less suitable, the first because they have poor keeping qualities owing to oxidation upon exposure to the air, the latter because they often fail to bring about a complete conversion of the diazo compound into azo dyestuff in the semi-wet development of diazotype material manufactured with diazo compounds according to the above definition and with a light-sensitive layer of normal composition.

In the diazotype process with semi-wet development phloroglucinol is the azo component most widely used. This compound can form mono-, bis- and tris-azo dyestuffs which are of different colours. The colours of the trisazo dyestuffs are darkest and those of the mono-azo dyestuffs lightest. As in practice a large visible image contrast in the developed diazotype copies is often desirable and the image contrast in general is larger according as the colour of the azo dyestuff formed during development is darker, the formation of as dark as possible an azo dyestuff is often desirable.

If larger than normal quantities of the acids or acid salts commonly used in diazotype materials, such as tartaric acid, citric acid, aluminium sulphate, and the like, are applied in the light-sensitive layers of one-component diazotype materials with diazo compounds according to the above definition, then, in semi-wet development with the said alkaline-reacting phloroglucinol developers which have been adapted to the higher acid content of the light-sensitive layer, dark azo dyestuffs, sometimes even—dependent on the diazo compound chosen—black azo dyestuffs, and thus copies with a greater image contrast, can be obtained.

However, owing to small deviations in the concentration of the developer and in the quantity of developer applied on the copy in semi-wet development, which deviations (hereinafter referred to as "development fluctuations") often occur in practice, e.g., in consequence of inaccuracies in the manufacture of the developing liquid, through evaporation of the latter during use, through irregularities in the operation of the developing apparatus, e.g., owing to vibrations, and to differences in developing speed, objectionable deviations in the shade of the azo dyestuffs are apt to appear. These deviations of shade are the more objectionable as the azo dyestuffs are darker. Especially with black azo dyestuffs such deviations are inconvenient.

In the one-component diazotype material according to the present invention the acid-reacting light-sensitive layer contains a quantity of alkali metal and/or ammonium orthophosphates in the amount of the stoichiometric

equivalent of at least 0.15 g. and at most 0.9 g. of  $P_2O_5$  per  $m^2$  (i.e., per square meter) of said material.

One-component diazotype material according to the invention yields, by semi-wet development with the said alkaline-reacting phloroglucinol developers, darker azo dyestuffs than corresponding diazotype material which contains no orthophosphate but only a larger quantity of one of the commonly used acids or acid salts. Moreover, the colours of the azo dyestuffs show considerably smaller deviations, or none at all, in consequence of the said deviations in the concentration and the application of the developer.

Quantities of orthophosphate which are the stoichiometric equivalents of less than 0.15 g. of  $P_2O_5$  per  $m^2$  are of little utility, because the effect of the invention is not achieved with them, or not to a sufficient degree. Quantities which are the stoichiometric equivalents of more than 0.9 g. of  $P_2O_5$  per  $m^2$  cause difficulties in the sensitization. The spreading of solutions containing such large quantities of phosphate over the surface of the diazotype material is not sufficiently uniform; they penetrate too far into some supports, such as paper.

The desired content of orthophosphate can be obtained by dissolving a suitable quantity of alkali metal or ammonium orthophosphate, e.g., primary sodium phosphate, in the sensitizing liquid, the magnitude of the quantity of sensitizing liquid which in the manufacture of the diazotype material is applied on the support per unit area naturally being taken into account.

The desired content of orthophosphate can also be obtained by treating the surface of the support to be sensitized, before the sensitization, with a solution of a suitable quantity of phosphate or by subjecting the sensitized surface to an after-treatment with such a solution. Primary, secondary or tertiary orthophosphates or mixtures of them can be used. Further, mixtures of orthophosphoric acid with alkali metal or ammonium salts of acids which are weaker than orthophosphoric acid may be employed. The phosphate-containing light-sensitive layer, however, must always show an acid reaction.

It is desirable in the production of diazotype layers to avoid volatile acids or acids with an offensive smell, such as formic acid, acetic acid, propionic acid or butyric acid. Accordingly, when using the above-mentioned mixtures of orthophosphoric acid with alkali metal or ammonium salts of weak acids, the use of salts of such volatile acids or acids with an offensive smell is also avoided.

The pH of the light-sensitive layer, or rather the pH of the light-sensitive surface (the light-sensitive layer of many diazotype materials, amongst others diazotype paper, is too thin for pH-determined inside the layer), is partly dependent on the pH and the acid and/or the buffer content of the support, but especially on the pH and the acid and/or the buffer content of the liquid(s), which is (are) used for the manufacture of the light-sensitive material. By providing for a suitable composition of this (these) liquid(s) it can easily be given a certain value. In practice this is not chosen below 2, since many diazotype materials, e.g., diazotype paper, become brittle at such a high degree of acidity of the light-sensitive layer and the sizing of the paper is adversely affected. It will preferably not be chosen higher than about 6.5 because the keeping qualities of the light-sensitive layers are then too small. The surface-pH of the light-sensitive layers of the common one-component diazotype materials in most cases is between 3.5 and 4.5.

In order to improve the keeping qualities of the light-sensitive material, a pH below 3.5 is sometimes chosen, particularly when above this pH value the keeping qualities would still leave much to be desired and if the application of stabilizers such as naphthalene-1,3,6-trisulphonic acid and its salts is not possible, for example owing to the formation of precipitates in the sensitizing liquids. If, however, stabilizers can be applied, a higher pH, e.g., between 4.5 and 6.5, may be chosen in many

cases. As the pH which the light-sensitive layer has before the development is to a certain extent also decisive for the formation of the azo dyestuff, it will have to be adapted somewhat to the coupling activity of the diazo compound used and to the developer to be used. The pH of the light-sensitive layer during the development, however, is much more important for the formation of the azo dyestuff.

Upon comparison of diazotype material according to the invention with corresponding diazotype material which contains instead of phosphate a larger quantity of the commonly used acids or acid salts, it therefore has to be taken into account that it is not necessary for the surface-pH which is measured for the comparable diazotype materials before the development to be exactly the same. The comparability is determined in the first place by the results of the development, in other words by the question of whether in the development the same quantity of diazo molecules is converted into azo dye-stuff in about the same time.

The surface-pH can easily be determined by wetting the light-sensitive surface locally with distilled water with the aid of the so-called surface-electrodes of an electric pH-meter that has been adjusted to the measurement, e.g. the surface glass electrode 6B 14/100 and the surface calomel electrode 6B 15/100 of the pH-meter type 6C of N.V. Electrofact, Amsterdam, Holland, in such a way that between the two electrodes via the wetted surface an electrical contact is effected, and by subsequently reading the deflection of the meter.

The inclusion of orthophosphate in light-sensitive layers of one-component diazotype materials employing the diazo compounds according to the above definition is not known.

One-component diazotype material is known in which a diazo film layer contains as diazo compound p,p'-tetrazo-o,o'-dianisidine and also contains a large quantity of primary sodium phosphate. The phosphate serves to prevent the bleeding of the azo dyestuff during bath-development, and can therefore be replaced by an equal quantity of common salt. In the semi-wet development of this material with the said alkaline-reacting phloroglucinol developers no favourable effect of the phosphate with regard to deviations in the shade of the azo dyestuffs owing to deviations in the concentration and the application of the developers is observed.

Another known one-component diazotype paper is that sensitized with the actively coupling 4-diazo-2,5-dieethoxy benzoylanilide, the light-sensitive layer of which contains a small quantity of primary sodium phosphate. This quantity is smaller than that which corresponds to 0.15 g. of  $P_2O_5$  per  $m^2$ . The paper is suitable for development with an acid, buffered phloroglucinol developer. In this case the deviations in shade owing to development fluctuations, as described above, do not arise. In the semi-wet development of this paper with the said alkaline-reacting phloroglucinol developers no favourable effect of the phosphate with regard to deviations in the shade of the azo dyestuffs owing to deviations in the concentration and the application of the developers is observed.

In order to avoid the disadvantageous consequences of development fluctuations in the semi-wet development of diazo film layers, it has been proposed to sensitize diazo film layers with a p-diazo-dialkylaminobenzene compound in which every alkyl group contains at least 4 and at most 7 C-atoms and the two alkyl groups together contain 10, 11 or 12 C-atoms and at most one of the two alkyl groups carries a side-chain at the  $\alpha$ -C-atom.

These diazo film layers contain very small quantities of the acids commonly used in the diazotype process such as tartaric acid, citric acid, and alum. The diazo compounds are not suited for the sensitization of some supports commonly used in the diazotype process, e.g. paper, because their solutions penetrate too far into them. They are also less light-sensitive than the diazo compounds

which can be applied in the diazotype material according to the invention.

Diazotype materials which have been sensitized with actively coupling diazo compounds, such as 4-diazo-2.5-dialkoxy-acylanilides, 4-diazo-2.5-dialkoxy-aryl-mercaptobenzene compounds, and 4-diazo-2.5-dialkoxy diphenyl compounds, and which are usually developed with acid, strongly buffered developers, can be developed, as is known, according to the semi-wet process with alkaline-reacting phloroglucinol developers, and may then yield azo dyestuff shades as pure or neutral and as dark as those obtained by development with the said strongly buffered developers, if their light-sensitive layer contains a large quantity of a saturated aliphatic dicarboxylic acid, in which the carboxyl groups are attached to carbon atoms which form part of a saturated hydrocarbon radical with at least 2 carbon atoms which may or may not be branched and may or may not be provided with other substituents, the dissociation constants of said acid being smaller than  $1 \times 10^{-4}$ . Examples of such acids are succinic acid, glutaric acid and adipic acid. Using these acids, development fluctuations in the semi-wet development of the last-mentioned diazotype materials with alkaline-reacting phloroglucinol developers have considerably less objectionable consequences than arise when acids such as citric acid, tartaric acid, alum, and the like are employed.

The use of large quantities of aliphatic saturated dicarboxylic acids in the light-sensitive layers of diazotype materials which have been sensitized with the same diazo compounds as those used in the diazotype materials according to the invention, does result indeed in the formation of darker azo dyestuffs in semi-wet development with alkaline-reacting phloroglucinol developers as mentioned above, and in decreased liability to development fluctuations, but both effects are smaller than those which are obtained according to the present invention. Moreover, diazotype material according to the present invention has better keeping qualities.

In the diazo compounds which are used in the diazotype material according to the invention it is not only the substituents in the phenyl radical carrying the diazo group, but also the other groups besides that phenyl radical which are attached to the tertiary nitrogen atom which affect the colour of the azo dyestuffs formed from the diazo compounds by semi-wet development. In general the azo dyestuffs are darker accordingly as the tertiary nitrogen atom carries heavier groups. Thus many diazo compounds of which the tertiary nitrogen atom carries two ethyl groups, when used in diazotype material according to the present invention, do not yield black-coloured, but lighter, more or less brown to dark brown azo dyestuffs upon development of the diazotype material with phloroglucinol developer. Corresponding diazo compounds with heavier alkyl groups, e.g. n-butyl groups, or with an aralkyl group, e.g. a benzyl group, on the tertiary nitrogen atom often yield fine black azo dyestuffs. Such diazo compounds, however, are often less readily soluble in the sensitizing liquids which are used for the manufacture of the diazotype material according to the present invention, while their light-decomposition products often cause rather serious discolouration of the diazotype copies. Both the said solubility and the said discolouration are worse accordingly as the quantity of phosphate used is larger.

Fine black azo dyestuffs, the colour of which remains practically unchanged when development fluctuations arise, are obtained with one-component diazotype material according to the present invention which contains a p-diazo-2.5-dialkoxy phenylmorpholine. The diazo compounds used in such one-component diazotype material do not have the disadvantages which corresponding diazo compounds with heavier groups on the tertiary nitrogen atom present.

One-component diazotype material sensitized with p-

diazo-2.5-diethoxy-phenylmorpholine is known. It does not contain orthophosphate.

The diazotype material according to the present invention may of course also contain mixtures of diazo compounds.

Furthermore it may contain the additives commonly used in one-component diazotype materials, such as stabilizers, e.g. naphthalene-1.3.6-trisulphonic acid or one of its salts, anti-discolouration agents, e.g. thiourea, means for improving the surface, e.g. fine particles of silica, aluminium oxide, synthetic resins or rice starch.

The diazo compounds used in the diazotype material according to the present invention can be prepared in several ways, e.g. as described in Belgian Patent No. 564,343. Compounds with an aralkoxy group can be prepared from o-nitro-phenyl-aralkyl ethers in the manner described in the said Belgian patent for the preparation of alkoxy compounds. Compounds with an aryloxy group can be prepared in a corresponding way from o-nitro-diphenyl ethers.

The following examples will serve to illustrate the invention:

*Example I*

White base-paper of weight 80 g.m.<sup>2</sup> as used for the diazo-type process is sensitized with a solution of:

13 g. of 4-di-n-propylamino-3-ethoxybenzene diazonium chloride, zinc chloride double salt  
40 g. of primary sodium phosphate (2 aq.)

25 2.5 g. of tartaric acid  
1 g. of boric acid  
20 g. of naphthalene-1.3.6-trisulphonic acid sodium salt  
30 cm.<sup>3</sup> of polyvinyl acetate dispersion Vinnapas H.60  
in 1000 cm.<sup>3</sup> of water

30 and dried.  
The sensitized surface contains approximately 0.38 millimole of diazo compound per m.<sup>2</sup> and a quantity of phosphate which is the stoichiometric equivalent of 0.18 g. of P<sub>2</sub>O<sub>5</sub> per m.<sup>2</sup>, and has a pH 3.85.

35 The light-sensitive side of a sheet of the diazotype paper thus prepared is covered with a sheet of tracing paper on which a pencil drawing has been made, and exposed in an exposure apparatus equipped with actinically fluorescent low-pressure mercury vapour lamps.  
40 Exposure is continued until, in the portions which are in contact with the blank parts of the drawing, only a small quantity of diazo compound is left.

45 The moment at which the exposure has to be terminated can be determined very well by visual observation (from the direction of the light-source, for instance) of the change of colour which occurs in the light-sensitive layer during the exposure. This moment is soon reached.

The latent diazotype copy thus obtained is developed by applying on its image surface a layer of approximately 8 g./m.<sup>2</sup> of a developing liquid of the following composition:

50 31 g. of thiourea  
15 g. of phloroglucinol  
55 1 g. of hydroquinone monosulphonic acid potassium salt  
2 g. of dibutylnaphthalene sulphonic acid sodium salt  
(commercially available under the name of Sorbit P)  
15 g. of sorbitol  
74 g. of potassium tetraborate (5 aq.)  
60 12.6 g. of potassium hydroxide  
in 1000 cm.<sup>3</sup> of water.

The developing liquid has a pH 9.8. The developed copy shows a strong black positive image on a uniform foggy background.

65 70 If the developing liquid is diluted, e.g. by addition of 200 cm.<sup>3</sup> of water, the copy developed with it shows an image which is less strong but still black.

If, instead of 40 g. of primary sodium phosphate, 12.5 g. of tartaric acid is used in the sensitizing liquid, a brown-black image is obtained with the above-mentioned devel-

oper, and a greenish black, incompletely developed, image with the diluted developer.

#### Example II

White base-paper of weight 80 g./m.<sup>2</sup> as used for the diazotype process is sensitized with a solution of:

13.5 g. of 4-(N-methyl-N-benzyl)amino-3-methoxybenzene diazonium chloride, zinc chloride double salt  
60 g. of primary sodium phosphate (2 aq.)  
3.5 g. of orthophosphoric acid  
0.8 g. of methylcellulose  
in 1000 cm.<sup>3</sup> of water  
and dried.

The sensitized surface contains approximately 0.38 millimole of diazo compound per m.<sup>2</sup> and a quantity of phosphate which is the stoichiometric equivalent of 0.29 g. of P<sub>2</sub>O<sub>5</sub> per m.<sup>2</sup>, and has a pH 3.6.

A sheet of the diazotype paper thus prepared is image-wise exposed as described in Example I. The moment at which the exposure has to be terminated can be observed very well and is soon reached.

The latent diazotype copy thus obtained is developed in a developing apparatus as described in Dutch Patent No. 67,009 at a speed of 5 m./min., 8.5 g./m.<sup>2</sup> of a developing liquid of the following composition being applied:

31 g. of thiourea  
6.5 g. of phloroglucinol  
6.5 g. of resorcinol  
2 g. of isopropylnaphthalene sulphonic acid sodium salt  
5 g. of sorbitol  
15 g. of saccharose  
53 g. of potassium tetraborate (5 aq.)  
9 g. of potassium hydroxide  
in 1000 cm.<sup>3</sup> of water.

The developing liquid has a pH 9.4. A strong black image on a foggy background is obtained.

When the developing speed in the above-mentioned developing apparatus is decreased to 3 m./min., the quantity of developer applied is reduced to 7 g./m.<sup>2</sup>. A copy developed at that speed shows a somewhat weaker, incompletely developed image, the azo dyestuff of which is somewhat greenish black in colour.

If, instead of 60 g. of primary sodium phosphate, 12.5 g. of citric acid is used in the sensitizing liquid, development at a speed of 5 m./min. yields a dark brown image and development at a speed of 3 m./min. a very incompletely developed green-brown image.

#### Example III

White base-paper of weight 80 g./m.<sup>2</sup> as used for the diazo-type process is pre-sensitized with about 10 g./m.<sup>2</sup> of the following liquid:

100 cm.<sup>3</sup> of colloidal silica dispersion Satessa 14  
2 g. of polyvinyl alcohol, Rhodoviol BS 10  
in 900 cm.<sup>3</sup> of water  
and dried.

The surface thus treated is sensitized with a solution of:

17 g. of 4-(N-2'-hydroxyethyl-N-benzyl)amino-3-methoxybenzene diazonium chloride, zinc chloride double salt  
40 g. of primary ammonium phosphate  
1.5 g. of tartaric acid  
30 cm.<sup>3</sup> of polyvinyl acetate dispersion, Vinnapas H.60  
in 1000 cm.<sup>3</sup> of water  
and dried.

The sensitized surface contains approximately 0.5 millimole of diazo compound per m.<sup>2</sup> and a quantity of phosphate which is the stoichiometric equivalent of 0.28 g. of P<sub>2</sub>O<sub>5</sub> per m.<sup>2</sup>, and has a pH 3.5.

A sheet of the diazotype paper thus prepared is image-wise exposed as described in Example I. The moment

at which the exposure has to be terminated can be observed very well and is soon reached.

The latent diazotype copy thus obtained is developed by applying approximately 9 g./m.<sup>2</sup> of the following developing liquid:

5 20 g. of sodium thiosulphate (5 aq.)  
15 g. of thiourea  
15 g. of phloroglucinol  
10 1 g. of hydroquinone monosulphonic acid potassium salt  
2 g. of Sorbit P  
2 g. of ethylene diamine tetraacetic acid, sodium salt  
25 25 g. of sodium carbonate  
in 100 cm.<sup>3</sup> of water.

The developing liquid has a pH 9.4. The developed copy shows a strong black positive image on a foggy background, which does not show deviations in shade due to vibrations and mechanical irregularities of the developing apparatus.

20 If, instead of 40 g. of primary ammonium phosphate, 27 g. of primary ammonium tartarate is used in the sensitizing liquid, considerable differences in azo dyestuff shade due to vibrations and mechanical irregularities of the developing apparatus are obtained, for example in the form of alternating black and brown-black lines in the azo dyestuff image.

#### Example IV

White base-paper of weight 80 g./m.<sup>2</sup> as used for the diazo-type process is sensitized with a solution of:

30 14 g. of 4-[N-methyl N-(naphthyl-1')methyl]amino-3-methoxybenzene diazonium chloride, zinc chloride double salt  
1 g. of aluminium sulphate (18 aq.)  
35 30 cm.<sup>3</sup> of polyvinyl acetate dispersion, Vinnapas H.60  
in 1000 cm.<sup>3</sup> of water

and dried.

On the light-sensitive surface a layer of approximately 10 g./m.<sup>2</sup> of the following liquid is applied:

40 40 g. of primary sodium phosphate (2 aq.)  
30 cm.<sup>3</sup> of polyvinyl acetate dispersion, Vinnapas H.60  
in 1000 cm.<sup>3</sup> of water.

45 After drying, the light-sensitive surface contains approximately 0.55 millimole of diazo compound per m.<sup>2</sup> and a quantity of phosphate which is the stoichiometric equivalent of 0.18 g. of P<sub>2</sub>O<sub>5</sub> per m.<sup>2</sup>. It has a pH 3.3.

A sheet of the diazotype paper thus prepared is image-wise exposed as described in Example I. The moment at 50 which the exposure has to be terminated can be observed very well and is soon reached.

The latent diazotype copy thus obtained is developed by applying approximately 8.5 g./m.<sup>2</sup> of the following developing liquid:

55 10 g. of thiourea  
15 g. of phloroglucinol  
2 g. of Sorbit P  
55 55 g. of tertiary sodium citrate (5 aq.)  
60 4.2 g. of sodium hydroxide  
in 1000 cm.<sup>3</sup> of water.

The developing liquid has a pH 9. The developed copy shows a strong black positive image on a foggy background.

65 When the concentration of the components of this developer has increased, for example in consequence of evaporation of the developer in the developing apparatus, to such an extent that the original volume of 1030 cm.<sup>3</sup> has decreased to about 750 cm.<sup>3</sup>, the development of a 70 copy on this light-sensitive material in an otherwise similar fashion results in an image of which the azo dyestuff has practically the same colour as that which is obtained with the developer of the normal concentration.

If, instead of 40 g. of primary sodium phosphate, 6 g. of aluminium sulphate (18 aq.) is used in the liquid

applied on the light-sensitive surface, a copy developed with the above-mentioned developer of the normal concentration shows a strong black image, but a copy developed with the developer after evaporation to 750 cm.<sup>3</sup> shows a brown-violet instead of a black image.

*Example V*

White base-paper of weight 80 g./m.<sup>2</sup> as used for the diazo-type process is sensitized with a solution of:

11 g. of 4-dimethylamino-3-phenoxybenzene diazonium chloride, zinc chloride double salt  
50 g. of primary potassium phosphate  
1.2 g. of orthophosphoric acid  
0.8 g. of methylcellulose  
in 1000 cm.<sup>3</sup> of water

and dried.

The sensitized surface contains approximately 0.5 millimole of diazo compound per m.<sup>2</sup> and a quantity of phosphate which is the stoichiometric equivalent of 0.41 g. of P<sub>2</sub>O<sub>5</sub> per m.<sup>2</sup> and has a pH 3.5.

A sheet of the diazotype paper thus prepared is image-wise exposed as described in Example I. The moment at which the exposure has to be terminated can be observed very well and is soon reached.

The latent diazotype copy thus obtained is developed as described in Example II.

The developed copy shows a grey-black positive image on a foggy background and shows only small variation of shade due to development fluctuations.

If, instead of 50 g. of primary potassium phosphate, 15 g. of aluminium sulphate (18 aq.) is used in the sensitizing liquid, considerable differences in azo dyestuff shade due to development fluctuations are obtained.

*Example VI*

A cellulose acetate layer of weight approximately 20 g./m.<sup>2</sup>, applied on natural tracing paper of weight approximately 80 g./m.<sup>2</sup>, is superficially hydrolyzed to a depth of approximately 4 $\mu$  and, after removal of the chemicals used for the hydrolysis by washing with water, is sensitized with a solution of:

24 g. of 4-dimethylamino-3-p-chlorophenoxy-6-chlorobenzene diazonium chloride, zinc chloride double salt  
80 g. of primary sodium phosphate (2 aq.)  
1.2 g. of orthophosphoric acid  
100 cm.<sup>3</sup> of ethanol 96%  
in 900 cm.<sup>3</sup> of water

and dried.

The light-sensitive hydrolyzed layer contains approximately 0.75 millimole of diazo compound per m.<sup>2</sup> and a quantity of phosphate which is the stoichiometric equivalent of 0.46 g. of P<sub>2</sub>O<sub>5</sub> per m.<sup>2</sup>, and has a surface pH 3.2.

A sheet of the diazotype material thus prepared is image-wise exposed as described in Example I. The moment at which the exposure has to be terminated can be observed very well and is soon reached.

The latent diazotype copy thus obtained is developed by applying approximately 8 g./m.<sup>2</sup> of the following developing liquid:

53 g. of sodium thiosulphate (5 aq.)  
20 g. of thiourea  
8 g. of borax  
7 g. of phloroglucinol  
7 g. of resorcinol  
1 g. of hydroquinone monosulphonic acid potassium salt  
2.5 g. of Sorbit P  
1.5 g. of ethylene-diamine tetraacetic acid, sodium salt  
27.5 g. of sodium carbonate  
in 1000 cm.<sup>3</sup> of water.

The developing liquid has a pH 9.4. The developed copy shows a brown-black image on a foggy background which shows little variation of shade due to development fluctuations.

If, instead of 80 g. of primary sodium phosphate, 19 g. of citric acid is used in the sensitizing liquid, considerable differences in azo dyestuff shade due to development fluctuations are obtained.

5 The copy produced according to this example can be used as an intermediate original for making further copies on diazotype paper.

*Example VII*

10 A baryta-coated paper of weight 125 g./m.<sup>2</sup> is sensitized with a solution of:

20 g. of 4-dimethylamino-3-benzyloxybenzene diazonium chloride, zinc chloride double salt  
56 g. of orthophosphoric acid, 50% by weight  
15 52.7 g. of tertiary sodium orthophosphate (12 aq.)  
2.5 g. of gum arabic  
30 cm.<sup>3</sup> of polyvinyl acetate dispersion, Vinnapas H.60  
in 1000 cm.<sup>3</sup> of water

20 and dried.

The sensitized surface contains approximately 0.7 millimole of diazo compound per m.<sup>2</sup> and a quantity of phosphate which is the stoichiometric equivalent of 0.38 g. of P<sub>2</sub>O<sub>5</sub> per m.<sup>2</sup>, and has a pH 4.3.

25 A sheet of the diazotype paper thus prepared is image-wise exposed as described in Example I. The moment at which the exposure has to be terminated can be observed very well and is soon reached.

The latent diazotype copy thus obtained is developed as described in Example II. The developed copy shows a grey-black positive image on a grey foggy background, which shows little or no deviation in shade due to vibrations and mechanical irregularities of the developing apparatus.

35 If, instead of the above-mentioned quantity of orthophosphoric acid and tertiary sodium orthophosphate, 16 g. of tartaric acid is used in the sensitizing liquid, the copy shows an image with considerable differences in azo dyestuff shade due to vibrations and mechanical irregularities of the developing apparatus, in the form of alternating brown and grey-black lines.

*Example VIII*

45 White base-paper of weight 80 g./m.<sup>2</sup> as used for the diazotype process is sensitized with a solution of:

12.5 g. of 4-(N-methyl-N-benzyl)amino-3-methoxy-6-bromobenzene diazonium chloride, zinc chloride double salt

50 70 g. of primary sodium orthophosphate (2 aq.)  
1.2 g. of orthophosphoric acid  
20 cm.<sup>3</sup> of polyvinyl acetate dispersion, Vinnapas H.60  
in 1000 cm.<sup>3</sup> of water

and dried.

55 The sensitized surface contains approximately 0.5 millimole of diazo compound per m.<sup>2</sup> and a quantity of phosphate which is the stoichiometric equivalent of 0.56 g. of P<sub>2</sub>O<sub>5</sub> per m.<sup>2</sup>, and has a pH 3.5.

A sheet of the diazotype paper thus prepared is image-wise exposed as described in Example I. The moment at which the exposure has to be terminated can be observed very well and is soon reached.

60 The latent diazotype copy thus obtained is developed as described in Example VI. The developed copy shows a grey-black positive image on a violet-grey foggy background, which shows little or no deviation in shade due to vibrations and mechanical irregularities of the developing apparatus.

If, instead of 70 g. of primary sodium orthophosphate, 70 22 g. of citric acid is used in the sensitizing liquid, the copy shows a dark-brown image on a red-brown foggy background with considerable differences in azo dyestuff shade due to vibrations and mechanical irregularities of the developing apparatus, for example in the form of 75 alternating green-brown, dark-brown and red-brown lines.

## 11

## Example IX

White base-paper of weight 80 g./m.<sup>2</sup> as used for the diazotype process is sensitized with a solution of:

24 g. of 4-morpholino-2,5-di-n-propoxybenzene diazonium chloride, zinc chloride double salt  
 60 g. of primary sodium orthophosphate (2 aq.)  
 3.5 g. of orthophosphoric acid  
 20 cm.<sup>3</sup> of polyvinyl acetate dispersion, Vinnapas H.60  
 in 1000 cm.<sup>3</sup> of water  
 and dried.

The sensitized surface contains approximately 0.45 millimole of diazo compound per m.<sup>2</sup> and a quantity of phosphate which is the stoichiometric equivalent of 0.23 g. of P<sub>2</sub>O<sub>5</sub> per m.<sup>2</sup>, and has a pH 3.4.

A sheet of the diazotype paper thus prepared is image-wise exposed as described in Example I. The moment at which the exposure has to be terminated can be observed very well and is soon reached.

The latent diazotype copy thus obtained is developed as described in Example II. The developed copy shows a strong black positive image on a foggy background which shows little variation of shade due to development fluctuations.

If, instead of 60 g. of primary sodium orthophosphate, 13 g. of citric acid is used in the sensitizing liquid, a dark violet-brown image is obtained.

## Example X

White base-paper of weight 80 g./m.<sup>2</sup> as used for the diazotype process is sensitized with a solution of:

14 g. of 4-morpholino-2,5-di-n-propoxybenzene diazonium chloride, zinc chloride double salt  
 20 g. of secondary sodium orthophosphate (2 aq.)  
 40 g. of primary sodium orthophosphate (2 aq.)  
 2 g. of citric acid  
 20 g. of naphthalene-1,3,6-trisulphonic acid, sodium salt  
 20 cm.<sup>3</sup> of polyvinyl acetate dispersion, Vinnapas H.60  
 in 1000 cm.<sup>3</sup> of water  
 and dried.

The sensitized surface contains approximately 0.45 millimole of diazo compound per m.<sup>2</sup> and a quantity of phosphate which is the stoichiometric equivalent of 0.35 g. of P<sub>2</sub>O<sub>5</sub> per m.<sup>2</sup>, and has a pH 5.4.

A sheet of the diazotype paper thus prepared is image-wise exposed as described in Example I. The moment at which the exposure has to be terminated can be observed very well and is soon reached.

The latent diazotype copy thus obtained is developed as described in Example II. The developed copy shows a strong black positive image on a foggy background which

## 12

shows little variation of shade due to development fluctuations.

If, instead of 20 g. of secondary sodium orthophosphate and 40 g. of primary sodium orthophosphate, 45 g. of tertiary sodium citrate and 15 g. of citric acid are used in the sensitizing liquid, considerable differences in azo dye-stuff shade due to development fluctuations are obtained.

We claim:

1. One-component diazotype material comprising a support carrying a light-sensitive layer containing a light-sensitive diazo compound in the absence of an azo coupling component, said light-sensitive layer having an acid reaction and said diazo compound being a p-amino benzene diazonium salt which has a greater coupling activity than p-diazo ethyl benzylaniline, which is derived from a tertiary amine with only one aryl radical attached directly to the tertiary nitrogen atom, and which carries in the 4-position the diazo group, in the 2-position a member selected from the class consisting of alkoxy, aryloxy and aralkoxy groups, and in the 5-position a member selected from the class consisting of a hydrogen atom, a halogen atom, a methyl group and an alkoxy group, the said light-sensitive layer containing a quantity of orthophosphate selected from the class consisting of alkali metal and ammonium orthophosphates in the amount of the stoichiometric equivalent of at least 0.15 g. and at most 0.9 g. of P<sub>2</sub>O<sub>5</sub> per square meter of said material.

2. One-component diazotype material according to claim 1, wherein the light-sensitive layer contains a diazonium salt of a p-diazo-2,5-dialkoxy-phenylmorpholine.

3. A process for the production of a diazotype print which comprises image-wise exposing a diazotype material as defined in claim 1 and developing the exposed material by the semi-wet method using a developer containing phloroglucinol.

4. One-component diazotype material according to claim 1, said diazonium salt being a diazonium salt of 4-di-n-propylamino-3-ethoxybenzene.

5. One-component diazotype material according to claim 1, said diazonium salt being a diazonium salt of 4-dimethylamino - 3 - p-chlorophenoxy - 6 - chlorobenzene.

6. One-component diazotype material according to claim 1, said diazonium salt being a diazonium salt of 4-morpholino-2,5-di-n-propoxybenzene.

## References Cited in the file of this patent

## UNITED STATES PATENTS

2,217,189 Sus \_\_\_\_\_ Oct. 8, 1940  
 50 2,405,523 Sease et al. \_\_\_\_\_ Aug. 6, 1946

## FOREIGN PATENTS

476,718 Canada \_\_\_\_\_ Sept. 4, 1951